

G. E. RENDALL.

## METHOD OF REDUCING ORES.

APPLICATION FILED NOV. 20, 1906.

932,175.

Patented Aug. 24, 1909.



## Inventor

George Frederick Rendall

## Witnesses

H. G. Dickerich  
R. A. Brewster

*By*  
Wiedersheim & Fairbanks  
Attorneys

# UNITED STATES PATENT OFFICE.

GEORGE FREDERICK RENDALL, OF NEW YORK, N. Y., ASSIGNEE TO AMERICAN REDUCTION COMPANY, A CORPORATION OF NEW JERSEY.

## METHOD OF REDUCING ORES.

932,175.

Specification of Letters Patent. Patented Aug. 24, 1909.

Application filed November 20, 1906. Serial No. 344,267.

*To all whom it may concern:*

Be it known that I, GEORGE FREDERICK RENDALL, a subject of Great Britain, residing in the city and county of New York, State of New York, have invented a new and useful Method of Reducing Ores, of which the following is a specification.

In a copending application having the same filing date, I have described and broadly claimed a novel and useful construction of an ore reducing furnace in which the necessity of employing fluxes is obviated, and my present invention consists of a novel method of reducing ores which can be carried out to advantage in a construction such as is illustrated and described in the above mentioned application.

One of the prominent features of my invention is the novel manner in which the reducing gas is employed, said gas performing a dual function, being first employed to calcine the ore and eliminate the sulfur and phosphorus contained therein, and afterward being combined with heated air to form the requisite combustion for heating the ore.

Another special feature of my invention is the manner in which the ore after treatment is discharged from the furnace without coming into contact with the atmosphere until sufficiently cooled and thus prevent any re-oxidation of the ore.

Another feature of my invention is the employment of the heated air externally generated around the gas retorts for mixing with gas, which has already been employed to calcine the ore, to produce the requisite combustion for heating the ore.

Another special feature of my invention is the manner in which the entire charge is subjected to gaseous treatment by the employment of an apertured member through which the reducing gas passes.

Other special features of my method will hereinafter more fully appear.

For the purpose of more clearly describing my invention, I have shown in the accompanying drawing, a sectional view of an ore reducing furnace which may be employed in carrying out my novel method.

1 designates a casing having a chamber 2 in which is located a plurality of gas retorts 3 provided with a source of heat 4. The gas producer or retort 3 is connected with a retort 5, the upper end of which forms an ex-

plosion chamber. The heated air in the chamber 2 is drawn therefrom through a conduit 6 by means of a suction device 7 and mixes and combines with the reducing gas which has acted on the charge, thereby removing the sulfur and phosphorus contents therein. The liability of the furnace being injured by the explosions, caused by the combining of the heated air and gas, is prevented by means of the counterbalanced cap 8. The ore is automatically fed from the furnace 9 into the retorts 5 and the ore in the furnace is heated by the combustion of the gas and the heated air, the gases passing through the ore and discharging into a gas receiver or container 10 in which they are collected for subsequent use. The ore is discharged from the retort 5 through a conduit 11 into a receptacle 12 from which all the air has been excluded.

In carrying out my method, I proceed as follows:—The ore is placed in the furnace and is heated by the combustion formed by the combination of the heated air generated externally of the gas retorts in the chamber 2, which is forced by a suction draft into contact with the reducing gas which has previously been employed to treat the charge in the retort. The ore thus treated in the furnace is fed or rabbled therefrom into the retort. The gas is led into said retort, which is preferably provided with an apertured bottom member in order that the entire charge will be subjected to gaseous treatment, and, after treating the charge, is combined with heated air to heat the charge in the furnace as above described. The ore is discharged from the retorts into closed receptacles or packages from which the air has been excluded to prevent any reoxidation.

When the ore is sufficiently cooled, it is treated magnetically or by concentration to eliminate all gangue which leaves the ore in an elementary condition. It is then placed in suitable packages, in the case of iron in metal cases, and then melted in a bath of molten material or in a cupola form of furnace. I attach much importance to this feature as it enables the ore to be mixed prior to melting with any desired compound and prevents small particles of fine material from escaping into the flues prior to fusion.

I attach a special importance to the method of admitting the gas to an apertured movable bottom in the furnace, whereby I am en-

abled to subject the entire charge to a gaseous treatment.

It will now be apparent that the gas is employed first, for treating the ore in a suitable retort and then for heating the ore with combustion produced by mixing with the gas a suitable proportion of heated air. It will be further apparent that after the ore has been calcined and treated with reducing gases, the same is cooled in a closed package so that there is no possibility of any reoxidization taking place.

Having thus described my invention, what I claim as new and desire to secure by Letters Patent, is:—

The method of reducing ores which consists in producing a reducing gas, leading

this gas into intimate contact with the charge in a retort, forcing heated air into an explosion chamber above the retort to unite 20 with gas passing from the charge, leading this gas to ore for a subsequent charge in a furnace communicating with the retort, discharging the charge into a closed receptacle from which the air has been withdrawn and 25 without admission of oxidizing atmosphere, sealing the receptacle and cooling the same, then mixing the ore with a desired compound prior to fusion, and then melting the ore in a bath of molten metal.

GEORGE FREDERICK RENDALL.

Witnesses:

HERBERT S. FAIRBANKS,  
C. D. McVAY.